

Feb. 16, 1965

B. HEROLD

3,169,928

COMPRESSION REFRIGERATION WORKING FLUID

Filed Feb. 24, 1959



INVENTOR:

Bern Herold  
by Deanne Shuey  
attorney

## 1

3,169,928

COMPRESSION REFRIGERATION WORKING  
FLUIDBernd Herold, Muhlenstrasse 53, Lüdinghausen, Germany  
Filed Feb. 24, 1959, Ser. No. 795,181  
3 Claims. (Cl. 252—68)

This invention relates to lubricating compositions for refrigerating machines and it has particular relation to compression refrigerating machines operated with halogenated hydrocarbons.

It has been known to use as refrigerating agents in refrigerating machines difluoromonochloromethane, difluorodichloromethane and methyl chloride. It has been also known that difluoromonochloromethane has certain essential advantages in comparison with the use of difluorodichloromethane which has been primarily used up to now. For example, difluoromonochloromethane is 1.6–1.7 times superior in its volumetric refrigerating capacity to difluorodichloromethane. Furthermore, in refrigerating machines operated with difluoromonochloromethane, lower cooling temperatures can be obtained in one step operation than with difluorodichloromethane under otherwise equal conditions.

However, it is a disadvantage that—in contrast to difluorodichloromethane—difluoromonochloromethane is not completely miscible with the mineral oils conventionally used as lubricating agents at low temperatures, as indicated by curves 1–3 of the appended drawing. The consequence of this is that expensive oil separators and oil return devices must be built in refrigerating machines operated with difluoromonochloromethane.

It has been known that oils having a naphthenic base (see curve 3 of the drawing) can be completely mixed with difluoromonochloromethane at lower temperatures than oils having a mixed naphthenic, or paraffinic base (see curves 1 and 2). However, the miscibility at low temperatures of difluoromonochloromethane with even very good oils having a naphthenic base is by far not sufficient for rendering dispensable the use of oil separators and oil return devices in refrigerating machines.

In order to overcome the above mentioned disadvantages occurring in the use of difluoromonochloromethane, instead of mineral oils, secondary silicic acid butyl esters (silicones) have been used as lubricating agents. It has been found that such esters are well miscible with difluoromonochloromethane so that the use of oil separators and oil return devices could be dispensed with. However, the use of said esters has the disadvantage that they are relatively expensive and their lubricating effect is lower than that of mineral oils.

It has now been unexpectedly found that synthetic oils of the type described hereinafter and obtained by condensation of olefins or halogen alkyls with aromatic hydrocarbons, are completely miscible with difluoromonochloromethane up to very low temperatures and that they meet the conventional requirements of stability to refrigerating agents. The stability of these synthetic products to difluorodichloromethane and to methyl chloride is likewise satisfactory and no copper plating occurs in their use. In mixtures of difluorodichloromethane with said synthetic products, the temperatures at which separation into the individual ingredients occurs are considerably lower than the corresponding separation temperatures in mixtures of the synthetic products with di-

## 2

fluoromonochloromethane. This has been observed also in the use of comparable conventional oils. The oils embodying the present invention can be universally utilized in refrigerating machines operated with difluoromonochloromethane, difluorodichloromethane and methyl chloride. The distillation residues obtained in the preparation of monoalkyl benzenes are particularly suitable for use according to the present invention.

Adjustment of the viscosity, flowing capacity at low temperatures, flash point, and average molecular weight, is carried out according to the present invention in such a manner that the requirements of DIN 51,503 as well as the requirement of complete miscibility with difluoromonochloromethane in all mixing proportions, up to temperatures of at least  $-25^{\circ}\text{ C.}$ , are met and no paraffin separations occur.

The synthetic lubricating oils of the present invention, or fractions of these oils, can be mixed with lubricating oils which, by themselves, are not, or not sufficiently, miscible for example with difluoromonochloromethane up to the desired temperatures in all mixing proportions. It has been found that by the admixture of oils of the present invention to other, e.g., conventional lubricating oils the miscibility minimum can be shifted in many variations up to the desired low temperatures.

In order to obtain the stability to refrigerating agents called for by DIN 51,503 and the low neutralization and saponification numbers likewise called for by said standard requirement, as well as in order to avoid copper-plating, it is contemplated according to the present invention to treat the oils of the invention with absorbing agents in order to reduce the resin content and the content of acid and/or saponifiable components in said oils.

## Example 1

A distillation residue obtained in the preparation of monoalkyl benzene from benzene and straight chain olefins consisting substantially of compounds having a chain length of  $C_{10}$ – $C_{13}$ , said residue boiling above  $210^{\circ}/12\text{ mm.}$  was subjected to a further vacuum distillation, in which 81% by volume of the residue subjected to distillation was obtained as distillate. After treatment with bleaching earth, this polyalkylated benzene distillate oil had the following characteristics:

|    |                                                                   |                                                         |
|----|-------------------------------------------------------------------|---------------------------------------------------------|
| 48 | Viscosity at $20^{\circ}\text{ C.}$ -----                         | 10.9° E.                                                |
|    | Viscosity at $50^{\circ}\text{ C.}$ -----                         | 3.5° E.                                                 |
|    | $d/20^{\circ}\text{ C.}$ -----                                    | 0.874.                                                  |
|    | Flash point -----                                                 | $213^{\circ}\text{ C.}$                                 |
| 50 | Solidifying point -----                                           | $-53^{\circ}\text{ C.}$                                 |
|    | Acid number -----                                                 | 0.01.                                                   |
|    | Saponification number -----                                       | 0.2.                                                    |
|    | Low temperature flowing capacity<br>according to DIN 51,568 ----- | $20\text{ mm.}/17\text{ sec. at }-25^{\circ}\text{ C.}$ |
| 55 | Stability to refrigerating agents -----                           | Over 96 hours.                                          |
|    | Miscibility with difluoromonochloromethane -----                  | See curve 4 of the drawing.                             |

## Example 2

A distillation residue obtained in the preparation of monoalkyl benzene from benzene and tetramer propylene, which boiled above  $210^{\circ}/12\text{ mm.}$ , was subjected to a further distillation under vacuum, in which 90% by volume of said residue were obtained as distillate. After

treatment with bleaching earth the polyalkylated benzene oil had the following characteristics:

|                                                             |                          |
|-------------------------------------------------------------|--------------------------|
| Viscosity at 20° C.                                         | 36.6° E.                 |
| Viscosity at 50° C.                                         | 5.0° E.                  |
| d/20° C.                                                    | 0.874.                   |
| Flash point                                                 | 175° C.                  |
| Solidifying point                                           | -34° C.                  |
| Acid number                                                 | 0.01.                    |
| Saponification number                                       | 0.1.                     |
| Flowing capacity at low temperature according to DIN 51,568 | 4 mm./60 sec. at -25° C. |
| Stability to refrigerating agents                           | Over 96 hours.           |

Mixtures of this oil with difluoromonochloromethane, which contained in one case 17.1 % and in a second case 10.3% of the oil, showed separation only at temperatures of -64° C. and below -65° C., respectively.

#### Example 3

A polyalkylated oil boiling above 150° C./12 mm. and obtained as distillation residue in the preparation of mono-alkyl benzene by reacting benzene with straight chain terminal olefins consisting mainly of compounds having a chain length of C<sub>10-13</sub>, and with chloroparaffins of similar chain length had—after treatment with bleaching earth—the following characteristics:

|                                                             |                             |
|-------------------------------------------------------------|-----------------------------|
| Viscosity at 20° C.                                         | 9.45° E.                    |
| Viscosity at 50° C.                                         | 2.7° E.                     |
| d/20° C.                                                    | 0.900.                      |
| Flash point                                                 | 208° C.                     |
| Solidifying point                                           | -50° C.                     |
| Acid number                                                 | 0.01.                       |
| Saponification number                                       | 0.2.                        |
| Flowing capacity at low temperature according to DIN 51,568 | 20 mm./13.1 sec. at -25° C. |
| Stability to refrigerating agents                           | Over 96 hours.              |

The separation or segregation temperatures of mixtures of difluoromonochloromethane containing (a) 15.3% and (b) 9.5% synthetic oil of this example, were at (a) -57° C. and (b) -65° C.

#### Example 4

A distillation residue boiling above 190° C./12 mm. and obtained in the preparation of monoalkyl benzene by reacting benzene with a dodecene, of the isobutene type, obtained by dimerization of n-hexane, is subjected to further distillation under vacuum, whereby about 75% by volume of the residue distilled, were obtained as distillate. After bleaching with bleaching earth, the polyalkylated benzene distillate oil had the following characteristics:

|                     |      |       |
|---------------------|------|-------|
| Viscosity at 20° C. | ° E. | 14    |
| Viscosity at 50° C. | ° E. | 3.1   |
| d/20° C.            |      | 0.862 |
| Flash point         | ° C. | 210   |
| Solidifying point   | ° C. | -44.5 |

A mixture of this oil with difluoromonochloromethane containing 13.6% of the oil did not show separation upon cooling to -70° C.

#### Example 5

A conventional commercial lubricating mineral oil of low viscosity for refrigerating machines was mixed in the proportion 1:1 with the alkylation residue distillate de-

scribed in the above Example 2. This mixture had the following characteristics:

|                                                             |                             |
|-------------------------------------------------------------|-----------------------------|
| Viscosity at 20° C.                                         | 13.7° E.                    |
| Viscosity at 50° C.                                         | 2.9° E.                     |
| d/20° C.                                                    | 0.884.                      |
| Flash point                                                 | 183° C.                     |
| Solidifying point                                           | -42° C.                     |
| Acid number                                                 | 0.05.                       |
| 10 Saponification number                                    | 0.1.                        |
| Flowing capacity at low temperature according to DIN 51,568 | 20 mm./52.7 sec. at -25° C. |

15 Mixtures of this oil with difluoromonochloromethane, which contained (a) 3.01% and (b) 12.1% of said oil, showed separation at (a) -51° C. and (b) -33° C.

#### Example 6

20 A highly viscous, conventional commercial lubricating mineral oil was mixed in the proportion of 30:70 with the alkylation residue described in the above Example 3. This mixture had the following characteristics:

|                                                             |                             |
|-------------------------------------------------------------|-----------------------------|
| Viscosity at 20° C.                                         | 11.6° E.                    |
| Viscosity at 50° C.                                         | 2.8° E.                     |
| d/20° C.                                                    | 0.901.                      |
| Flash point                                                 | 198° C.                     |
| 30 Solidifying point                                        | -49° C.                     |
| Acid number                                                 | 0.06.                       |
| Saponification number                                       | 0.1.                        |
| Flowing capacity at low temperature according to DIN 51,568 | 20 mm./22.6 sec. at -25° C. |

Miscibility with difluoromonochloromethane is shown in curve 5 of the drawing.

40 The term "bleaching earth" is used herein to denote materials which have strong absorbent capacity and are used, among others, for the purification of oils by absorption, such as fuller's earth, bentonite, Florida bleaching earth and the like.

45 The preparation of synthetic oils in the above described manner, e.g., by condensation from benzene and olefin hydrocarbons, has been known by itself from the art and is described, for example, in the German patents No. 767,299 and 895,588.

50 The temperatures stated herein are centigrade, and the parts mentioned are by weight, if not otherwise stated. The term "terminal olefin" is used herein to denote olefins, in which the double bond is located between the last two C-atoms of the chain.

55 The residues mentioned in the above examples are preferably distilled up to a temperature of about 330° C. under a vacuum of about 12 mm.

It will be understood from the above that this invention is not limited to the specific materials, steps, conditions 60 and other details specifically described above and can be carried out with various modifications without departing from the scope of the invention as defined in the appended claims.

65 It will be also understood that the appended drawing illustrates the miscibility of difluoromonochloromethane with various mineral oils at various temperatures (curves 1, 2, 3) and the miscibility of synthetic oils embodying the present invention (curves 4 and 5) as indicated by the legends in the drawing.

70 The abbreviation "DIN" is used herein to denote the standards published by the "Deutsche Industrie Normung" (German Industrial Standardization). The abbreviation "d" is used to denote "density" and the abbreviation "E" is used to denote "Engler" degrees of viscosity.

What is claimed is:

1. A compression refrigeration working fluid consisting essentially of

- (1) from 75% to 97% of a halogenerated aliphatic hydrocarbon refrigerant, and,
- (2) from 3% to 25% of a lubricating oil consisting essentially of,
  - (a) 0% to 50% of a petroleum mineral oil, and
  - (b) 100% to 50% of a polyalkylated benzene distillation residue having,
    - (i) an initial boiling point between 150° C. @ 12 mm. Hg and 210° C. @ 12 mm. Hg,
    - (ii) a final boiling point of about 330° C. @ 12 mm. Hg,
    - (iii) a viscosity at 20° C. between 9° and 37° E.,
    - (iv) a viscosity at 50° C. between 2° and 5° E.,

said working fluid remaining single phase at -25° C.

2. The compression refrigeration working fluid of claim 1 wherein said refrigerant is selected from the group consisting of difluoromonochloromethane, difluorodichloromethane, and methyl chloride.

3. The compression refrigeration working fluid of claim 2 wherein said refrigerant is difluoromonochloromethane.

References Cited in the file of this patent

UNITED STATES PATENTS

|    |           |                |       |               |
|----|-----------|----------------|-------|---------------|
| 5  | 2,138,775 | Towne          | ----- | Nov. 29, 1938 |
|    | 2,141,593 | Clarke et al.  | ----- | Dec. 27, 1938 |
|    | 2,424,956 | Reiff et al.   | ----- | July 29, 1947 |
| 10 | 2,477,382 | Lewis          | ----- | July 26, 1949 |
|    | 2,810,769 | Sanford et al. | ----- | Oct. 22, 1957 |
|    | 3,092,981 | Begeman et al. | ----- | June 11, 1963 |

FOREIGN PATENTS

|               |       |               |
|---------------|-------|---------------|
| Australia     | ----- | May 18, 1951  |
| Australia     | ----- | July 23, 1958 |
| France        | ----- | Apr. 21, 1958 |
| Germany       | ----- | May 2, 1952   |
| Germany       | ----- | Nov. 5, 1953  |
| Great Britain | ----- | July 16, 1952 |
| Great Britain | ----- | Oct. 29, 1958 |